

J. A. HEANY,  
INCANDESCENT ELECTRIC LAMP,  
APPLICATION FILED JULY 29, 1916.

1,399,722.

Patented Dec. 6, 1921.

*Fig. 1.*



*Fig. 2.*



*Fig. 3.*



*Inventor:*  
John Allen Heany  
*by* *James Goldbaugh & Meier*  
*Atty.*

# UNITED STATES PATENT OFFICE.

JOHN ALLEN HEANY, OF NEW YORK, N. Y.

## INCANDESCENT ELECTRIC LAMP.

1,399,722.

Specification of Letters Patent.

Patented Dec. 6, 1921.

Application filed July 29, 1916. Serial No. 111,997.

*To all whom it may concern:*

Be it known that I, JOHN ALLEN HEANY, a citizen of the United States, residing in the city of New York, county of New York, 5 and State of New York, have invented certain new and useful Improvements in Incandescent Electric Lamps; and I do hereby declare the following to be a full, clear, and exact description of the invention, such 10 as will enable others skilled in the art to which it appertains to make and use the same.

This invention relates to incandescent electric lamps and has for its object to provide an improved glower for use therein and also an improved method of making the glower.

In its preferred form, the glower comprises a base of porous refractory material, 20 such, for example, as zirconium oxid, thorium oxid, magnesium oxid, or the like, or mixtures of these compounds impregnated wholly or in part with a highly refractory metal, such as tungsten, titanium, molybdenum, vanadium, tantalum or the like having a higher fusing point than the platinum group, or mixtures of these metals. Although the size and shape of the glower are immaterial, so far as the broader aspects 25 of the invention are concerned, it is preferably made substantially cylindrical in shape, of relatively short length and large diameter, as compared with the filament of the ordinary strung lamp, for the purpose of 30 reducing the convection losses.

The invention is illustrated in the accompanying drawing, in which:—

Figure 1 is a front elevation of an incandescent electric lamp having a glower 40 mounted therein constructed in accordance with the invention.

Fig. 2 is a transverse vertical section through the porous refractory base before the same is impregnated with the refractory metal; and

Fig. 3 is a transverse vertical section through the glower showing the porous base partly impregnated with the refractory metal.

The exact manner of mounting the glower in the lamp is immaterial, but it is preferably mounted as shown in Fig. 1, in which the usual bulb is indicated at 1 with which there is associated the ordinary threaded 50 metallic base 2. The base 2 is electrically connected with the lead wires 3 and 4 which

serve to support the glower, denoted generally by the reference character A. The bulb 1 is preferably filled with an inert gaseous medium, such as nitrogen, mercury vapor 60 or the like, having low thermal conductivity for the purpose of keeping down the convection losses, and capable of preventing to as great an extent as possible, evaporation 65 of the glower.

The porous base shown at a in Figs. 2 and 3 is, as above stated, made of some refractory compound, such as zirconium oxid, thorium oxid or a similar porous refractory material of very low conductivity, 70 but which possesses great strength even at the operating temperature. It is obvious that if desired, several of these compounds may be used in conjunction to form the base. In the manufacture of the glower, 75 the refractory compound or compounds are made into a plastic mass molded to the proper shape, and then baked to the required degree. This baking may be effected at extremely high temperature and for such 80 a length of time that the base will be completely shrunk to its final form, or else the base may be baked only to such an extent that it is rendered sufficiently hard to be handled and the final baking may be postponed until after the base is impregnated 85 with the refractory metal.

The material used for impregnating the base may be either metal in a finely divided state, a solution of the metal, or a compound of the metal. If a metallic compound is used, the compound is converted into metal. If, for instance, it be desired to impregnate the base with a refractory metal, such as tungsten, a solution may be 90 made of ammonium tungstate which is soluble in water. The porous base may be steeped in this solution, dried and the solution converted to metallic tungsten by heat and hydrogen gas. A solution of colloidal 100 ammonium paratungstate may also be used and after the porous base is steeped in this solution, it is dried and treated by heat and hydrogen gas which reduces the tungsten compound to metallic tungsten. It is also 105 possible to impregnate the porous refractory base with a pseudo colloidal metal, such as those produced by arcing in various liquids.

It is obvious that the entire body of the 110 refractory base a may be impregnated with the refractory metal, or only a portion there-

of may be impregnated, as shown at *b* in Fig. 3. It is also obvious that the porous base may be subjected to as many steeping operations as desired, in order to vary the 5 content of refractory metal in the final glower. A very small amount of metal may be incorporated in the refractory base by utilizing a weak solution of the metallic compound, so it is, therefore, evident that 10 the process is very flexible, in that the quantity of metal incorporated in the base may be readily varied to vary the conductivity of the glower. If it be desired to impregnate the porous base with a metallic alloy, 15 the base may be treated with solutions of two or more metallic compounds.

After the steeping operation of the porous base, the same is baked at a high temperature and for a sufficient length of time 20 to shrink the glower to its final form before it is mounted in the bulb, provided this baking operation is not performed before the base is impregnated with the refractory metal. In the latter instance, care 25 should be taken to preserve the porous nature of the base.

The improved glower may be made relatively short and of large diameter to reduce the convection losses without sacrific-

ing its strength or materially increasing its 30 conductivity, because the support *a* possesses great strength, even at the highest temperatures at which the lamp is operated, and the current in traversing the glower passes only through the conductive refractory 35 metal incorporated in the base. The refractory metal, therefore, serves as the resistor and heats the base of refractory compound to incandescence.

Although the glower is represented in the 40 drawing as being of solid cylindrical shape, it is obvious that it can be made in various other shapes.

What I claim is:—

The process of making a glower for incandescent electric lamps, which consists in molding into desired shape a plastic mass of highly refractory material, treating said mass to produce a strong porous body, impregnating the said body with a solution 50 of a metallic compound, the metal of which incandesces at the temperature at which platinum volatilizes, and then reducing the compound to metal by heating the glower in the presence of hydrogen. 55

In testimony whereof I affix my signature.

JOHN ALLEN HEANY.